

## UNITED STATES PATENT OFFICE

AUGUSTUS B. KINZEL, OF BEECHHURST, LONG ISLAND, NEW YORK, ASSIGNOR TO  
ELECTRO METALLURGICAL COMPANY, A CORPORATION OF WEST VIRGINIA

## METHOD OF NITRIDING METALS

No Drawing.

Application filed May 26, 1931. Serial No. 540,207.

My invention relates to the production of nitrided layers on metals by heating the metals in the presence of suitable nitrogen-containing agents, such as ammonia. It has 5 particular reference to an improved method of forming such nitrided layers.

The object of my invention is to provide a means by which the action of nitriding gases on metal articles is accelerated and 10 intensified, so as to reduce the time required to produce a case of given hardness or thickness.

The case hardening of alloys is useful as a means of forming hard wear-resisting 15 surfaces on articles which are to be subject to abrasion. In order to form adherent and non-brittle cases, and to prevent distortion of the articles undergoing treatment, it is customary to carry out the production of 20 nitride cases at low temperatures, usually of the order of 460° C. to 580°. To produce satisfactory cases at these low temperatures it has been found advisable to alloy with the material to be treated small 25 amounts of a promoting agent such as aluminum or vanadium. The procedure customarily followed consists, essentially, in heating the alloyed articles in a muffle or similar externally-fired furnace in the presence 30 of a nitriding agent. When this procedure is followed a heating period of from 12 to 20 hours is required to form a useful case, the time of heating increasing with a decrease in temperature employed. Such 35 prolonged heating is expensive, and at the present time forms a large part of the total cost of the nitriding process. It is evident that a saving in the time of heating required to produce a case of the desired hardness 40 and thickness would result in a material reduction in the cost of nitriding.

I have discovered that a remarkable increase in the speed of production of a nitride case by contact with a nitriding gas 45 occurs when the customary process is so modified that the heating is done directly by the action of electric currents electromagnetically induced in, or in the surface of, the articles under treatment, instead of by 50 the indirect heating heretofore used. When

the article to be nitrided is thus heated by induction, the rate of hardening is increased to a surprising degree, as will be demonstrated below.

According to my invention, the heating 55 may be done by any suitable means whereby electromagnetically induced electric currents are produced in the articles of sufficient magnitude to cause a rise of temperature of the surface of those articles to the temperature 60 at which the nitriding reactions are to be carried out. It should be noted that if high voltages are used in induction heating, the electromagnetically induced currents are largely restricted to the surface of the 65 article. Similarly, the nitriding gas may be any suitable gas of this description, and may be applied to the article by any feasible means or method.

In the preferred form of my invention 70 the articles are placed in a chamber containing a gaseous nitriding agent and surrounded by a coil carrying high-frequency electric currents. The chamber is preferably so constructed and equipped that a continuous 75 slow flow of the nitriding gas through the chamber may be used. By this arrangement, high-frequency currents are induced in the metal articles, whereby the surface temperature of those articles is raised to 80 the desired reaction temperature. Under these conditions a definite case is produced in materially shorter time than under conditions heretofore employed in the art. For example: Several pieces of steel, alloyed 85 with small amounts of chromium and aluminum, were heated for four hours at a temperature of 460° C. by means of electric currents of high frequency induced in the test pieces in an electric induction furnace. 90 During this heating period a slow stream of ammonia gas was passed over the steel pieces. At the end of this treating period the samples showed a definite, hard and adherent case. The average hardness of the 95 samples before this treatment was about 98 Rockwell, while their average hardness after this treatment was about 115 Rockwell, sufficiently hard to scratch glass with ease; the average depth of case produced was 100

from ten to fifteen thousandths of an inch. Pieces of similarly alloyed steel, heated in a stream of ammonia for four hours at the same temperature in a muffle furnace according to the commonly known procedure, showed no appreciable hardening, as was to be expected from common experience in the art.

The particular furnace used in the above test is a standard 20 k. w. condenser-type high-frequency induction furnace utilizing a frequency of approximately 10,000 cycles per second. It will be understood that the use of a standard furnace, or of this stated frequency, is not essential to secure improvement in the art of nitriding as now practiced with an externally-fired furnace. Any practical means of directly heating the articles by electric currents electromagnetically induced therein, as well as the use of any frequency that will cause a rise of temperature of the surface of the articles to the reaction temperature, gives the improvement sought in this invention. It is to be pointed out however that the best results are to be secured by the use of higher frequencies, such as those of the order used in the examples given above.

It will be evident that numerous modifications of the method as described above may be made without departing from the spirit of my invention as disclosed in this specification and the appended claims.

I claim:

- 35 1. The method of nitriding metal articles which comprises heating the articles in the presence of a nitriding agent by means of high-frequency electric currents electromagnetically induced in said articles.
- 40 2. The method of nitriding metal articles which comprises heating the articles in the presence of a nitriding agent by means of high-frequency electric currents induced in said articles.
- 45 3. The method of nitriding ferrous articles which comprises heating the articles in the presence of ammonia by means of high-frequency electric currents induced in said articles.
- 50 4. The method of nitriding ferrous articles which comprises heating the articles in the presence of ammonia by means of high-frequency electric currents electromagnetically induced in the surface of said articles.
- 55 5. The method of nitriding ferrous articles containing nitride-promoting agents such as chromium, aluminum, or vanadium, which comprises heating the articles in the presence of ammonia by means of electric currents of a frequency of the order of 10,000 cycles per second induced in said articles.

In testimony whereof, I affix my signature.

AUGUSTUS B. KINZEL.